# EUROPEAN PATENT SPECIFICATION

(11) **EP 0 385 448 B1**
(45) Date of publication and mention of the grant of the patent: **04.08.1993**
(21) Application number: 90103924.8
(22) Date of filing: 28.02.1990
(51) Int. Cl.: C23C 28/00

(54) **Method of coating metal assembly including aluminum member**
Verfahren zur Beschichtung von Werkstücken mit Aluminium
Procédé pour le revêtement d'un ensemble métallique contenant des pièces en aluminium

(30) Priority: 28.02.1989 JP 48953/89; 13.07.1989 JP 181983/89
(43) Date of publication of application: 05.09.1990
(73) Proprietor: NIPPON PAINT CO., LTD., Osaka-shi Osaka-fu (JP)
(72) Inventor: Oshiba, Toshiharu, Itami-shi, Hyogo-ken (JP); Yamamoto, Hisataka, Setagaya-ku, Tokyo (JP)
(74) Representative: Hansen, Bernd, Dr. Dipl.-Chem.

(56) References cited:
- DE-A- 1 180 216
- DE-A- 3 616 567
- GB-A- 2 169 618
- US-A- 4 650 696

## Description

The present invention relates to a method of coating a metal assembly including at least one aluminum part and steel parts, particularly to a method of coating assembled metal members for automobile bodies.

In the coating of automobile bodies constituted by different metal members such as steel parts, zinc-plated steel parts, zinc alloy-plated steel parts and aluminum parts, since most parts are constituted by steel parts, only aluminum parts occupying small areas are coated after stamping, degreasing and chemical treatment. The reasons therefor are that since chemical coatings for steel parts constituting the automobile bodies are formed by zinc phosphate chemicals, aluminum is dissolved away from the aluminum parts by the chemicals, and accumulated in the treating solutions, and that when an amount of aluminum accumulated in the chemical treating solutions exceeds a certain level, the formation of chemical coatings on the steel surfaces is inhibited.

It was proposed by Japanese Patent Publication No. 45-16566 to remove the accumulated aluminum by adding fluoric acid for precipitating the dissolved aluminum to the chemical coating agents. However, it is difficult to control the exact amount of fluoric acid necessary for precipitating aluminum, and the precipitated aluminum forms sludge such as cryolite Na₃AlF₆ and elpasolite NaK₂AlF₆ . The sludge should be removed from the chemical treatment bath frequently, or the chemical treatment bath should be renewed frequently.

Jitsumu Hyomen Gijutsu (Metal Finishing Practice) Vol. 35, No. 1, 1988 discloses a method of coating assembled members consisting of aluminum parts and steel parts in which the aluminum parts and the steel parts are treated separately in their exclusive treatment lines and the treated aluminum parts and the steel parts are combined in a final stage. However, in this method, the exclusive lines are necessary for both of the aluminum parts and the steel parts, and the treated aluminum parts and the steel parts should be handled very carefully in assembling. In addition, painted parts may have slightly different finish colors.

In addition to the above problems, when aluminum parts are subjected to deep drawing by stamping, a large amount of a lubricating oil having a high viscosity should be used to impart good workability to the aluminum parts, thereby preventing cracks, scratches and strains. However, it is generally difficult to remove this lubricating oil, requiring much time and labor. Therefore, aluminum parts which can be stamped without using lubricating oils are desired.

Accordingly, an object of the present invention is to provide a method of coating a metal assembly including at least one aluminum part in which the aluminum part and the other parts, namely steel parts can be treated simultaneously, thereby effectively coating the aluminum member for automobile bodies, etc.

As a result of intense research in view of the above object, the inventors have found than an aluminum part coated with a conductive primer is highly resistant to a treatment with chemical solutions which is necessary for chemically treating steel parts, and that the aluminum part coated with a conductive primer can be easily stamped to provide deep-drawn products, etc. without using lubricating oils. The present invention is based on these findings.

Thus, the invention as defined in independent claims 1 and 5 comprises a method of coating a metal assembly of Al parts with uncoated and/or zinc or zinc-alloy coated steel parts comprising the steps of :
degreasing of the Al part;
applying a conductive primer to said aluminum part:
baking the primer to form an organic coating layer;
combining said aluminium part with the steel part and providing the resulting assembled parts with chemical coatings or with chemical coatings and and electrodeposition coatings.

Preferred embodiments of the processes are defined in the dependent claims 2-4 and 6. According to a further embodiment the method of coating a metal assembly comprises also the step of conducting the formation of an intermediate coat and/or top coat after forming electrodeposition coatings.

The metal assembly to which the coating method of the present invention can be applied is constituted of at least one aluminum part and at least one other steel part . A typical combination comprising aluminum parts and steel parts (including zinc-plated steel parts). One combination is at least one aluminium part and at least one steel part. Specific combinations of metal parts to be assembled are exemplified as follows:

### 1. Aluminum parts coated with a conductive primer.

Steel parts (coated with or without a conductive primer).

A metal assembly of these plates is provided with chemical coatings and electrodeposition coatings, optionally followed by the formation of an intermediate coat and/or a top coat.

### 2. Aluminum parts coated with a conductive primer.

Steel parts which may be subjected to chemical coating.

After the aluminum parts are stamped, they are assembled with steel parts and then provided with an intermediate coat and/or a top coat.

### 3. Aluminum parts coated with a conductive primer.

Steel parts.

After the aluminum parts are stamped, they are assembled with steel parts and then provided with chemical coatings.

These assembled parts are used for example for automobile bodies or electric appliances. In some applications, plastic members may be combined with aluminum parts and steel parts.

The conductive primer which may be used in the present invention comprises:
(A) a bisphenol-type epoxy resin having a number average molecular weight of 300 to 100,000, in an amount of 30 weight % or more on a solid basis;
(B) at least one hardener selected from a polyisocyanate and a blocked polyisocyanate in an amount of one-tenth to 2 times the weight of the above epoxy resin;
(C) fumed silica having an average particle size of 0.1 to 100 milli-µm, in an amount of 5 to 50 weight % on a solid basis; and
(D) a ketone solvent in an amount of 40 weight % or more based on the total weight of the primer.

The solid content of the conductive primer is 10 to 50 weight %, which makes it possible to form a thin, uniform, conductive primer layer with excellent corrosion resistance, high conductivity in electrodeposition coating, improved formability, and excellent adhesion to an electrodeposition coating layer.

Usable as the binder resin (A) is a bisphenol-type epoxy resin soluble in an organic solvent and having a number average molecular weight of 300 to 100,000, which is excellent in water resistance, alkali resistance, and good adhesion to a substrate material as well as a top coat. Examples are the epoxy resins represented by the formula:
in which R is H or CH₃; A is 〉C(CH₃)₂, -CH₂-, -O-,

Particular preference is given to the epoxy resin wherein A is 〉C(CH₃)₂, having a number average molecular weight of 1,000 to 5,000, because of extremely improved anti-corrosion properties.

If the number average molecular weight of the epoxy resin is less than 300, it is unable to get a high polymer when reacted with a polyisocyanate, making the resulting conductive primer layer deficient in anti-corrosive properties. On the other hand, when it is more than 100,000, a cross-linking degree decreases, providing the resulting conductive primer layer with poor anti-corrosive properties.

In the conductive primer layer used in the present invention, the above bisphenol-type epoxy resin (A) should be 30 weight % or more on a solid basis of the conductive primer layer, because, if otherwise, the resulting conductive primer layer is likely to be brittle and have poor adhesion after stamping.

The hardener (B) used in the present invention is selected from the group consisting of polyisocyanates and blocked polyisocyanates.

Examples of the polyisocyanates are aliphatic or alicyclic diisocyanates including hexamethylene diisocyanate, isophorone diisocyanate, hydrogenated diphenyl methane diisocyanate and the like; aromatic diisocyanates including tolylene diisocyanate, diphenyl methane-4,4'-diisocyanate and the like, triisocyanates as adducts of 1 mol of trimethylol propane and 3 mol of either one of the above-mentioned diisocyanates, trimers of hexamethylene diisocyanate, trimers of tolylene diioscyanate and the like.

As the blocked polyisocyanates, any of the above-mentioned polyisocyanates blocked with blocking agents may be used. Such blocking agents must be compounds capable of reacting with an isocyanate group and forming addition products which are stable at a room temperature but dissociated at a high temperature encountered at a baking stage, thereby making the isocyanate group free. Examples of the blocking agents are lactam blocking agents such as ε-caprolactam and γ-butyrolactam; oxime blocking agents such as methyl ethyl ketoxime and cyclohexanone oxime; alcohol blocking agents such as methanol, ethanol and isobutyl alcohol; phenol blocking agents such as phenol, p-t-butyl phenol and cresol; and β-diketone blocking agents such as ethyl acetoacetate, methyl acetoacetate, acetyl acetoacetate, dimethyl malonate and diethyl malonate.

From the aspect of dissociation at a relatively low temperature, particular preference is given to methyl ethyl ketoxime and β-diketones.

The above-mentioned hardener (B) is contained in the conductive primer in an amount of one-tenth to 2 times the weight of the epoxy resin (A) on a solid basis.

The epoxy resin (A) and the hardener (B) react with each other at a relatively low baking temperature in a short period of time, for example, at a maximum temperature of about 100°C or more, preferably at 120°C to 200°C, in 5 to 60 seconds.

If the mixing ration of (B)/(A) is less than 1/10, the cross-linking reaction is insufficient, resulting in poor corrosion resistance of the conductive primer layer. On the other hand, if the ratio (B)/(A) is more than 20/10, the conductive primer layer are provided with poor water resistance, alkali resistance and adhesion to an overlying coat. Particularly preferable mixing ration of the hardener (B) to the epoxy resin (A) is such that NCO equivalent of the hardener (B)/OH equivalent of the epoxy resin (A) is within a range of 0.1/1 - 1.0/1. Under these conditions, excellent anti-corrosion properties can be achieved.

The above-mentioned hardener (B) may be used together with a resol-type phenyl resin, if desired. This is especially effective in accelerating the film-forming reaction at a relatively low baking temperature, for example, at a maximum temperature of 100°C to 130°C.

Particularly preferable resol-type phenol resins are the compounds of the formula:
wherein n is an integer of 0 to 4; W is -CH₂- or -CH₂-O-CH₂-; R is CH₃, H, or

Such a resol-type phenol resin is preferably added in an amount up to 10 times the weight of the hardener (B) on a solid basis. If the weight ratio of the phenol resin/hardener (B) is more than 10/1, alkali resistance of the resulting conductive primer layer is likely to be lowered.

In the present invention, fumed silica (C) having an average particle size of 0.1 to 100 milli-µm serves to provide the primer layer with electric conductivity, because ions can pass through pores generated by the fumed silica in the primer layer in the processes of chemical coating and electrodeposition coating. If the average particle size of the silica is less than 0.1 milli-µm, the conductive primer layer is insufficient not only in electric conductivity but also in adhesion to an overlying layer and alkali resistance. On the other hand, when the average particle size of the fumed silica exceeds 100 milli-µm, the corrosion resistance of the resulting conductive primer layer is lowered.

The fumed silica (C) amounts to 5 to 50 weight %, preferably 15 to 30 weight %, on a solid basis of the conductive primer. Heretofore, such a large quantity of fumed silica has not been used, because it makes the conductive primer highly viscous. However, this problem has been solved by the use of particular ketone solvent (D).

When the fumed silica (C) is less than 5 weight % on a solid basis of the conductive primer, the corrosion resistance of the resulting conductive primer layer becomes poor. On the other hand, if it exceeds 50 weight %, adhesion properties of the conductive primer layer after stamping tend to be undesirably decreased.

The epoxy resin (A), the hardener (B) and the fumed silica (C) are dissolved or dispersed in a ketone solvent. The ketone solvent (D) should be 40 weight % or more to adjust the solid content of the conductive primer to 10 to 50 weight %.

If the solid content of the conductive primer is less than 10 weight %, it is uneconomical because too much solvent is consumed. On the other hand, if it exceeds 50 weight %, it is hardly possible to form a thin, uniform conductive primer layer.

Preferred examples of the ketone solvents (D) are methyl isobutyl ketone, acetone, cyclohexanone and isophorone. If desired, additional solvents other than the ketone solvent may be used together therewith. However, solvents reactive with polyisocyanates, e.g. water and alcohol, should be avoided.

From the viewpoint of formability of precoated aluminum parts, the conductive primer may further contain 0.1 to 10 weight %, based on the conductive primer, of such lubricants as polyolefins, carboxylates, metal carboxylates, polyalkylene glycols, molybdenum disulfide, silicone compounds and fluorinated compounds. Particularly preferable lubricants are polyethylene waxes having densities of 0.94 or more, molecular weights of 1,000 and 10,000 and acid values of 15 KOH mg/g or less.

To enhance the electric conductivity of the conductive primer, conductive material powder such as carbon black, graphite powder, zinc oxide powder, titanium oxide powder, aluminum powder, copper powder, etc. may be added in proper proportions.

If desired, the conductive primer may further contain known anti-corrosive pigments (e.g. chromate pigments, especially zinc chromate, lead chromate and barium chromate, phosphate pigments and plumbate pigments), extender pigments (e.g. carbonate pigments and silicate pigments), coloring pigments (e.g. titanium oxide and carbon black), anti-corrosive agents (e.g. amine compounds and phenolic carboxylic acids and dispersion stabilizers.

The conductive primer used in the present invention forms an organic coating layer which is electrically conductive for the purpose of the present invention. The term "conductive" used herein means that the aluminum parts coated with the conductive primer can be provided with chemical coatings and electrodeposition coatings, namely meaning that electric conductivity can be achieved through the conductive primer in the process of electrodeposition coating, etc. The reasons therefor may be considered that since the conductive primer layer is thin and porous, electrodeposition coating composition can be attracted to the aluminum parts via the conductive primer.

In addition, in a case where stamping such as deep drawing is conducted, the conductive primer provides the aluminum parts with excellent workability, thereby making it unnecessary to use lubricating oils. This is an outstanding advantage because the process of removing lubricating oils from the stamped aluminum parts can be omitted. In addition, when the aluminum parts are combined with the steel parts, it is preferable to use a conductive primer for providing the same coating appearance to the aluminum parts and the steel parts.

To achieve the object of the present invention sufficiently, the aluminum parts are coated with the conductive primer on one or both sides thereof, and they conveyed to an automobile body manufacturing line, etc., where the aluminum parts is stamped and combined with steel parts for subsequent treatments. However, in an alternative method, after assembling the aluminum parts with the steel parts, the conductive primer may be applied to the assembled parts by spraying, and then baked.

The conductive primer is usually applied to the aluminum parts in a dry film thickness of 10 µm or less. When the dry film thickness exceeds 10 µm, the conductive primer shows high insulation, making it difficult to provide it with chemical coatings and electrodeposition coatings. Accordingly, the resulting caoted aluminum parts have a poor corrosion resistance, impact resistance and workability. The preferred dry film thickness of the conductive primer layer is 0.1-5 µm. When it is lower than 0.1 µm, the conductive primer-coated aluminum parts is vulnerable to erosion in a zinc phosphate treatment bath, permitting a large amount of aluminum to be dissolved into the zinc phosphate treatment bath. In addition, in the case of stamping, the aluminum parts tends to have cracks and strains. The more preferred dry film thickness of the conductive primer layer is 0.5-3 µm.

The chemical coating can be conducted by using known coating chemicals. The preferred coating chemicals for the purpose of the present invention are zinc phosphate chemicals which contain zinc ions, phosphate ions, hydrochloric ions, nitrite ions, and, if necessary, nickel ions, nitrate ions, chlorine ions in proper proportions. A typical example of the coating chemicals consists essentially of about 0.4 to about 1 g/l of zinc, about 5 to about 40 g/l of phosphate, about 0.01 to about 0.2 g/l of nitrite and about 2 to about 5 g/l of chlorate. Such coating chemicals suitable as primers for forming electrodeposition coatings are exemplified in Japanese Patent Laid-Open No. 55-145180.

The coating chemicals may be applied to the aluminum parts and the Steel parts separately or in combination. It should be noted that the coating chemicals are not necessarily indispensable for the aluminum parts, but that the coating chemicals can provide the aluminum parts with better corrosion resistance. When an assembly of the aluminum parts coated with the conductive primer and steel parts for constituting automobile bodies, is immersed in a chemical treatment bath of zinc phosphate chemicals, the precoated aluminum parts is not eroded by the chemical treatment bath so that substantially no aluminum sludge is formed in the bath.

Next, the assembled members are provided with electrodeposition coatings. The electrodeposition coating composition may be either one of a cation type and an anion type which are known in the art. A uniform electrodeposition coating layer having a good appearance can be formed on the precoated aluminum parts and the chemically treated steel parts.

If necessary, an intermediate coat and/or a top coat can be formed on the assembled members thus treated. As an alternative method, without subjecting the aluminum parts coated with the conductive primer to chemical coating with zinc phosphate chemicals, electrodeposition coating can be conducted, optionally followed by the formation of an intermediate coat and/or a top coat.

Incidentally, if oils, dusts, strains, etc. are attached to the conductive primer layers, it is preferable that they are removed by solvents, etc. before subsequent treatments.

Preferred examples of the coating process according to the present invention are as follow:
(1)
   (a-1) Aluminum parts are degreased by a known method.
   (a-2) Conductive primer is roll-coated and baked at a maximum temperature of 100-160°C for 20 seconds.
   (b-1) Assembling the aluminum parts with steel parts to provide automobile bodies,
   (b-2) Forming chemical coatings.
   (b-3) Forming electrodeposition coatings.
   (b-4) Forming an intermediate coat and/or a top coat.
(2)
   (a-1) Aluminum parts are degreased by a known method.
   (a-2) Conductive primer is roll-coated and baked at a maximum temperature of 100-160°C for 20 seconds.
   (b-1) Stamping.
   (b-2) Assembling the aluminum parts with steel parts to provide automobile bodies, etc.
   (b-3) Forming electrodeposition coatings.
   (b-4) Forming an intermediate coat/ a top coat.
(3)
   (a-1) Aluminum parts are degreased by a known method.
   (a-2) Conductive primer is roll-coated and baked at a maximum temperature of 100-160°C for 20 seconds.
   (b-1) Stamping.
   (b-2) Assembling the aluminum parts with steel parts to provide automobile bodies,
   (b-3) Forming an undercoat by spraying.
   (b-4) Forming an intermediate coat and/or a top coat.

In the above processes, the steps (a-1), (a-2) may be conducted in aluminum-working lines, and the steps (b-1), (b-2) ... may be conducted in assembly lines of automobile bodies.

The present invention will be described in further detail by means of the following Examples.

### Example 1

The following coating process is conducted:
(a-1) Preparing aluminum parts (degreased by a known method).
(a-2) Applying an epoxy resin-type conductive primer (NIPPE METALCOAT P19 CLEAR, manufactured by Nippon Paint Co., Ltd.) to the aluminum parts in a dry film thickness of 0.5 µm.
(a-3) Stamping the precoated aluminum parts (a-2).
(b-1) Assembling the stamped aluminum parts (a-3) and a stamped steel plate (cold-rolled Steel parts) to provide an automobile body.
(b-2) Forming chemical coatings.
   (i) Degreasing with alkali by immersing the automobile body in a 2-% RIDOLINE SD 400 (manufactured by Nippon Paint Co., Ltd.) solution at 60°C for 3 minutes.
   (ii) Rinsing with water.
   (iii) Surface adjusting by immersing the automobile body in a 0.1-% FIXODINE 5N-10 (manufactured by Nippon Paint Co., Ltd.) solution at 25°C for 30 minutes.
   (iv) Forming coating chemicals by immersing the automobile body in zinc phosphate chemicals (GRANODINE DP 3000, manufactured by Nippon Paint Co., Ltd.) solution having a concentration:$\text{Concentration=} \frac{\text{Total Acid}}{\text{Free Acid}} \text{=} \frac{\text{18}}{\text{0.9}} \text{=20}$ at 50°C for 2 minutes.
   (v) Rinsing with water.
   (vi) Final rinsing (if necessary) by spraying at 0.1-% DEOXYLITE 41 (manufactured by Nippon Paint Co., Ltd.) solution at 20°C for 1 second.
   (vii) Rinsing with pure water by spraying at 20°C for 1 second.
   (viii) Drying at 150°C for 2 minutes.
(b-3) Forming electrodeposition coatings.
   Cation electrodeposition paint: POWERTOP U-600, manufactured by Nippon Paint Co., Ltd.
   - Voltage applied:: 200 V.
   - Applying time:: 3 minutes.
   - Bath temperature:: 30°C.
   - Baking:: 185°C, 20 minutes.
   - Dry film thickness:: 25 µm.
(b-4) Forming intermediate coat with ORGA P-41 GRAY, manufactured by Nippon Paint Co., Ltd.
   - Baking:: 140°C, 30 minutes.
   - Dry film thickness:: 35 µm.
(b-5) Forming top coat with:
   (1) SUPERLAC M-80 METALLIC, manufactured by Nippon Paint Co., Ltd., and
   (2) SUPERLAC O-50 CLEAR, manufactured by Nippon Paint Co., Ltd.
   by a wet-on wet coating process.
   - Baking:: 140°C, 30 minutes.
   - Dry film thickness:: 20/35 µm.

Various properties are evaluated, and the results are shown in Table 1.

### Example 2

The same coating process as in Example 1 is conducted except for changing the dry film thickness of NIPPE METALCOAT P19 CLEAR to 5 µm. Various properties are evaluated, and the results are shown in Table 1.

### Example 3

The following coating process is conducted:
(a-1) Preparing aluminum parts (degreased by a known method).
(b-1) Applying an epoxy resin-type conductive primer (NIPPE METALCOAT P19 CLEAR, manufactured by Nippon Paint Co., Ltd.) to the aluminum parts in a dry film thickness of 1 µm.
(b-2) stamping the precoated aluminum parts.
(b-3) Assembling the stamped aluminum parts and a stamped steel plate (cold-rolled Steel parts) to provide an automobile body.

The formation of coating chemicals, electrodeposition coatings, an intermediate coat and a top coat are conducted in the same process as in Example 1. Various properties are evaluated, and the results are shown in Table 1.

### Comparative Examples 1-4

An assembly of aluminum parts and an Steel parts is coated as follows:

### [1] Treatment of aluminum parts

(1) Coating them with various amounts of lubricating oils.
(2) Stamping the aluminum parts at various stamping levels.
(3) Degreasing with alkali by immersing the stamped Aluminum parts in a 1-% RIDOLINE 53 (manufactured by Nippon Paint Co., Ltd.) solution at 60°C for 1 minute.
(4) Rinsing with water.
(5) Forming chemical coatings by immersing in 2-% chromate chemicals (ALODINE 1200, manufactured by Nippon Paint Co., Ltd.) at 40°C for 30 seconds.
(6) Rinsing with water.
(7) Drying.
(8) Forming electrodeposition coatings in the same process as in Example 1.

### [2] Treatment of Steel parts

(1) Coating chemical
   (i) Degreasing with alkali by immersing the steel parts in a 2-% RIDOLINE SD400 (manufactured by Nippon Paint Co., Ltd.) solution at 60°C for 3 minutes.
   (ii) Rinsing with water.
   (iii) Surface adjusting by immersing the steel parts in a 0.1-% FIXODINE 5N-10 (manufactured by Nippon Paint Co., Ltd.) solution at 25°C for 30 minutes.
   (iv) Forming coating chemicals by immersing the Steel parts in a zinc phosphate chemicals (GRANODINE DP 3000, manufactured by Nippon Paint Co., Ltd.) having a concentration:$\text{Concentration=} \frac{\text{Total Acid}}{\text{Free Acid}} \text{=} \frac{\text{18}}{\text{0.9}} \text{=20}$ at 50°C for 2 minutes.
   (v) Rinsing with water.
   (vi) Final rinsing (if necessary) by spraying a 0.1-% DEOXYLITE 41 (manufactured by Nippon Paint Co., Ltd.) solution at 20°C for 1 second.
   (vii) Rinsing with pure water by spraying at 20°C for 1 second.
   (viii) Drying at 150°C for 2 minutes.
(2) Forming electrodeposition coatings in the same process as in Example 1.

### [3] Assembling the aluminum parts and the steel parts.

### [4] Forming an intermediate coat/a top coat on the assembled plates.

Various properties are evaluated in the same process as in Example 1, and the results are shown in Table 2.

As described above in detail, by the coating method of the present invention, a metal assembly including at least one aluminum part member and at least one steel part can be provided with chemical coatings and electrodeposition coatings without suffering from the erosion of the aluminum parts. In addition, the aluminum parts coated with the conductive primer can be stamped to any shape, such as a deep-drawn shape without using a lubricating oil. This is greatly advantageous in terms of productivity because the operation of removing a lubricating oil from the stamped aluminum parts usually takes a lot of time and labor.

## Claims

1. A method of coating a metal assembly of Al parts with uncoated and/or zinc or zinc-alloy coated steel parts comprising the steps of :
degreasing of the Al part;
applying a conductive primer to said aluminium part and
baking the primer to form an organic coating layer;
combining said aluminium part with the steel part and
providing the resulting assembled parts with chemical coatings and electrodeposition coatings.

2. The method according to claim 1, further comprising the step of conducting the formation of an intermediate coat and/or top coat after forming electrodeposition coatings.

3. The method according to claim 1, further comprising the step of conducting chemical coatings on the aluminium part before applying the conductive primer thereto.

4. The method according to claim 1, further comprising the step of stamping the aluminium part coated with said conductive primer before combining it with the steel part.

5. A method of coating a metal assembly of Al parts with uncoated and/or zinc or zinc-alloy coated steel parts comprising the steps of:
degreasing of the Al part;
applying a conductive primer to said aluminium part and baking the primer to form an organic coating layer;
stamping said aluminium part;
combining the stamped aluminium part with the steel part and then providing the resulting assembled parts with chemical coatings.

6. A method according to one or more of the preceeding claims wherein the thickness of the conductive primer, expressed as dry film thickness, is 0.1 to 10 µm.

## Patentansprüche

1. Verfahren zur Beschichtung einer Metallzusammenstellung aus Al-Teilen mit unbeschichteten und/oder zink- oder zinklegierungsbeschichteten Stahlteilen, umfassend die folgenden Schritte:
Entfetten des Aluminiumteils;
Aufbringen einer leitenden Grundierung auf dieses Aluminiumteil und
Brennen der Grundierung zur Bildung einer organischen Überzugsschicht;
Kombinieren des Aluminiumteils mit dem Stahlteil und Versehen der resultierenden zusammengesetzten Teile mit chemischen und galvanischen Überzügen.

2. Verfahren gemäß Anspruch 1, weiterhin umfassend den Schritt der Bildung einer Zwischenschicht und/oder Oberschicht nach der Bildung von galvanischen Überzügen.

3. Verfahren gemäß Anspruch 1, weiterhin umfassend den Schritt der Bildung von chemischen Überzügen auf dem Aluminiumteil vor dem Aufbringen der leitenden Grundierungsschicht darauf.

4. Verfahren gemäß Anspruch 1, weiterhin umfassend den Schritt des Stanzens des Aluminiumteils, das mit dieser leitenden Grundierung beschichtet wurde, bevor es mit dem Stahlteil kombiniert wird.

5. Verfahren zur Beschichtung einer Metallzusammenstellung aus Aluminiumteilen mit unbeschichteten und/oder zink- oder zinklegierungsbeschichteten Stahlteilen, umfassend folgende Schritte:
Entfetten des Aluminiumteils;
Aufbringen einer leitenden Grundierung auf dieses Aluminiumteil und Brennen der Grundierung zur Bildung einer organischen Überzugsschicht;
Stanzen des Aluminiumteils;
Kombinieren des gestanzten Aluminiumteils mit dem Stahlteil und dann Versehen der resultierenden zusammengesetzten Teile mit chemischen Überzügen.

6. Verfahren gemäß einem oder mehreren der vorhergehenden Ansprüche, worin die Dicke der leitenden Grundierung, ausgedrückt als die Dicke eines trockenen Films, 0,1 bis 10 µm beträgt.

## Revendications

1. Procédé de revêtement d'un assemblage métallique de pièces d'aluminium et de pièces d'acier non revêtues et/ou revêtues de zinc ou d'alliage de zinc, comprenant les étapes consistant à :
- dégraisser la pièce d'aluminium;
- appliquer un primaire conducteur sur cette pièce d'aluminium; et
- cuire le primaire pour former une couche de revêtement organique;
- associer cette pièce d'aluminium à la pièce d'acier et munir les pièces assemblées obtenues de revêtements chimiques et de revêtement par électrodéposition.

2. Procédé selon la revendication 1, comprenant en outre l'étape consistant à former une couche intermédiaire et/ou une couche de finition après avoir formé des revêtements par électrodéposition.

3. Procédé selon la revendication 1, comprenant en outre l'étape consistant à effectuer le revêtement par voie chimique sur la pièce d'aluminium avant d'appliquer sur celle-ci le primaire conducteur.

4. Procédé selon la revendication 1, comprenant en outre l'étape consistant à estamper la pièce d'aluminium revêtue de ce primaire conducteur avant de l'associer à la pièce d'acier.

5. Procédé de revêtement d'un assemblage métallique de pièces d'aluminium avec des pièces d'acier non revêtues et/ou revêtues de zinc ou d'alliage de zinc, comprenant les étapes consistant à :
- dégraisser la pièce d'aluminium;
- appliquer un primaire conducteur sur cette pièce d'aluminium; et
- cuire le primaire pour former une couche de revêtement organique;
- estamper cette pièce d'aluminium;
- associer la pièce d'aluminium estampée à la pièce d'acier, puis munir les pièces assemblées obtenues de revêtements par des produits chimiques.

6. Procédé selon l'une ou plusieurs des revendications précédentes, dans lequel l'épaisseur du primaire conducteur, exprimée par l'épaisseur du film sec, est de 0,1 à 10 µm.
